

March 15, 1938.

F. A. WALES

2,111,377

ART OF COATING ALUMINUM

Filed Nov. 14, 1935

2 Sheets-Sheet 1

FIG. 1.



FIG. 2.



INVENTOR.

*Fred A. Wales.*

BY

*Dike, Calmer & Gray*

ATTORNEYS.

March 15, 1938.

F. A. WALES

2,111,377

## ART OF COATING ALUMINUM

Filed Nov. 14, 1935

2 Sheets-Sheet 2



*INVENTOR.*

INVENTOR.

Dick, Calver & Gray

*ATTORNEYS.*

## UNITED STATES PATENT OFFICE

2,111,377

## ART OF COATING ALUMINUM

Fred A. Wales, Detroit, Mich.

Application November 14, 1935, Serial No. 49,647

3 Claims. (Cl. 204—1)

The present invention relates to the art of coating aluminum or aluminum alloys or articles formed therefrom, and particularly to improvements in the method of and apparatus for forming such coatings, particularly coatings of the so-called "oxide" type.

Such coatings on aluminum or aluminum alloys are commonly recognized as being formed chiefly of  $Al_2O_3$ ,  $SO_3$ , and  $H_2O$ , and are formed as a plurality of laminated layers which vary as to thickness, hardness and porosity. Such coatings have been formed by processes heretofore known to the art by making the aluminum or aluminum alloy an anode in an electrolytic cell having sulfuric acid as the electrolyte. The coatings are formed upon the passage of direct current electrical energies through the cell and are formed on the aluminum or the aluminum alloys which form the anode in the cell. The direct current used in such processes is of the order of twelve to eighteen volts and of from six to twenty amperes per square foot of material undergoing treatment. A cathode, electrically connected in the circuit, forms the other contact with the electrical circuit and is placed in the electrolyte. In certain embodiments, such cathode frequently was the tank, and the current flowed between the cathode and the anode through the electrolyte and caused the growth of the so-called "oxide" coating at the anode. In using such processes for the formation of the oxide coatings on aluminum or aluminum alloy articles, such for example as pistons for use in internal combustion engines, I have discovered that the coating formed by the processes of the prior art was not satisfactory in such fields due particularly to the large variations in fineness of grain structure, the irregularity as to size and distribution of pores, the extreme variations in hardness between the respective layers, and the relatively high cost of processing and of the apparatus for use therewith.

The process and apparatus of the present invention has as its principal object to provide a coating for aluminum or aluminum alloys, or articles formed therefrom, the coating being superior to coatings previously known and characterized by having a very dense fine grained laminated structure. The various layers exhibit substantially uniform hardness characteristics and are permeated with very small and substantially uniform pores between the particles of the coating.

It is a further object of the present invention to provide a process and apparatus for producing

a protective coating on aluminum or aluminum alloys, or articles formed therefrom, which is particularly, but not exclusively, adapted to produce the improved coatings on pistons formed of aluminum or aluminum alloys for use in internal combustion engines or similar purposes.

A further object of the present invention is to provide a process for the production of protective coatings on aluminum or aluminum alloys, or articles formed therefrom, in which the cost of operation and of the equipment has been reduced over similar costs of prior art processes and equipment, and which, while being more economical than processes and equipment of the prior art, produces coatings which are superior to the coatings produced by the prior art.

It is a further object of the present invention to provide an apparatus for use in forming protective coatings on aluminum or aluminum alloys, or articles formed therefrom, which is a portable self-contained unit.

Other objects of the present invention will appear in the following description and appended claims. One preferred form of apparatus embodying the present invention is shown by way of example in the accompanying drawings forming a part of this specification wherein like reference characters designate corresponding parts in the several views, and in which

Fig. 1 is a view in perspective of an apparatus which is adapted to be used in connection with the present process and embodied in the form of a self-contained portable unit.

Fig. 2 is a front view in elevation of the apparatus of Fig. 1 showing the enclosing cover in closed position.

Fig. 3 is an end view in elevation of the apparatus shown in Fig. 2.

Fig. 4 is a sectional view taken along the line 4—4 of Fig. 2 in the direction of the arrows.

Before explaining in detail the present invention it is to be understood that the invention is not limited in its application to the details of construction and arrangement of parts illustrated in the accompanying drawings, since the invention is capable of other embodiments and of being practiced or carried out in various ways. Also, it is to be understood that the phraseology or terminology employed herein is for the purpose of description and not of limitation, and it is not intended to limit the invention claimed herein beyond the requirements of the prior art.

The apparatus shown in the drawings comprises a casing 10 which is mounted upon a supporting rack 11, which may be provided with a

5 plurality of casters 12 to permit moving the entire unit from place to place about a plant. The casing 10 is divided interiorly to form a rinse tank 13 and a tank 14, which is provided with a lead or other non-corrosive lining 15 and is adapted to contain the electrolytic bath.

10 Mounted on one end of the framework 11 is a bracket 16 on which is mounted an electric motor 17 which drives a fan 18 of the blower type. An air pump 19, preferably of the pulsating type, is also driven by the motor 17 and is connected by means of the conduit 20 with a series of perforated pipes 21 extending across the bottom of the lead-lined tank 14. Air is supplied to the pipes 21 and is discharged therethrough to keep the electrolyte agitated during operation of the apparatus. The fan or blower 18 is connected by means of a duct 22 with the hooded upper part of the tank 14 (Fig. 4) and 15 serves to ventilate the apparatus while in operation.

20 During the operation of the apparatus, a hood or cover 23 is placed in the closed position, as shown in Fig. 4. The cover 23 prevents fumes given off during the carrying out of the process from escaping into the atmosphere, thus functioning as a collection hood from which the collected fumes are drawn through the duct 22 and are thereafter discharged through a stack (not shown), which is connected with a discharge opening 24 on the blower 18.

25 As shown in Fig. 4, the lead lining 15 forming the tank 14 is spaced apart from the casing 10 in such a manner as to provide a duct 25 which extends about all sides of the lead lining 15 inside the casing 10. The duct 25 communicates with the interior of the tank 13, into which may be placed a suitable temperature controlling fluid mass which will flow through the chamber 13 30 and around the duct 25 surrounding the lead lining 15 of the tank 14. By varying the temperature of the fluid medium in the tank 13, the temperatures within the tank 14 may be controlled within definite predetermined limits.

35 40 The fluid is fed into the tank 13 through a suitable conduit 26 which is operatively connected with the source of fluid supply and the level is maintained in the tank 13 by means of a waste or outlet pipe 27 which acts as an overflow pipe when the fluid reaches the top thereof. If water is used as the fluid temperature control medium in the tank 13, and its temperature is not sufficiently low to control the temperature of the tank 14, a cake of ice or other refrigerant 45 may be placed therein and so refrigerate the fluid which runs through the tank and around the chamber 25. During the operation of the apparatus, the tank 13 functions also as a rinse tank and the aluminum or aluminum alloys or other articles which have been treated in the treating tank may be rinsed in the tank 13 after the coating has been formed thereon.

50 55 Electrical energy is supplied to the tank 13 by means of a transformer 30 which is suitably mounted on the framework 11, preferably at a point adjacent the bottom of the tank 13. The transformer operates on alternating electrical current and in a preferred embodiment has a rated capacity of 200 amperes and 24 volts. The 60 transformer is of a conventional design adapted for use either on 110 volts or 220 volts, and is provided with a series of taps through which the current may be drawn to be passed to the bath, such current to have controlled and varying 65 voltages up to 24 volts.

60 65 A suitable control panel 31 is electrically connected with the transformer 30 and acts to provide the connections through which the current flows to the electrolytic bath. Electrical connections are provided between the transformer 30 through the control panel 31 with bus bars 32 which extend crosswise of the tank 14. The articles to be treated, such for example as aluminum or aluminum alloy pistons 33, are provided with a suitable clamp 34 which is electrically connected with and engages one of the bus bars 32 to suspend the article being treated into the electrolyte in the tank 14. In this manner the articles to be treated are connected through the electrolytic bath in a parallel series so that the flow of electricity is through the bus bars 32, the clamps 34, the article 33, through the electrolytic bath to the article 33, its clamp 34, and the bus bar 32. This method of connection is contrary to conventional methods in that the tank or bath 70 remains neutral, whereas in prior known processes the bath or tank forms the other connection with the electrical current and only the article being treated forms the anode thereof. In the present apparatus, with the use of alternating current, the articles 33 alternately form the anode and the cathode of the current flow and on the 110 volt, 60 cycle, line this alternation occurs sixty times each second, but will vary, however, with variations in the cycles of the alternating current.

75 80 A valve 35 is provided in the casing 10 and communicates with the duct 25 to permit withdrawal of fluid temperature control mediums therefrom.

85 90 The foregoing described apparatus, while being particularly adapted to the process of the present invention, is also adaptable (with slight changes, particularly as to its electrical circuit) for use in conventional processes known to the art, and as such, by reason of the temperature control provided in the electrolytic bath and in the portability of the unit, produces results which are desirable and which are superior to the apparatus previously known to the art, although it is my belief that using such apparatus with conventional processes will not produce the satisfactory results produced by the practice of my improved process therein.

95 100 The improved process of the present invention proceeds in part upon my discovery that a superior type of coating may be formed either on aluminum or aluminum alloys or articles formed therefrom, and can be provided by using the aluminum or aluminum alloy or article formed therefrom as both the anode and the cathode of the electrical circuit flowing through the electrolytic bath. The change from anode to cathode is preferably a successively occurring change which will be brought about in relatively rapidly alternating sequence. The process also proceeds upon my discovery that such successively and rapidly alternating electrical changes in the character of the aluminum or aluminum alloy during the coating operation can best be effected by utilizing various voltages of 60 cycle alternating current, beginning at approximately 12.5 volts and increasing the voltage of the electrical flow during the coating operation to 24 volts at a time when the temperature of the bath is definitely controlled between limits of approximately 69° to 74° F.

105 110 In carrying out the present process, I provide an electrolytic bath in the tank by using commercial grades of sulphuric acid in concentrations 75

of 13% by weight in aqueous solution. At least two pieces of the aluminum or aluminum alloy or article formed therefrom are electrically connected, one with each side of the line supplying the electric current to the electrolytic bath and from the anode and cathode respectively of the cell resulting from the immersion of the articles in the electrolyte.

The operation is started at a voltage of the lower order, preferably from 9 to 12½ volts, which is increased as the operation proceeds, to the higher range of voltages, preferably from 20 to 24 volts. The temperature of the bath is preferably maintained from approximately 69° F. to approximately 73° F. by the use of a suitable circulating temperature control medium surrounding the tank in which the operation is being carried on. The treatment and processing is complete within time intervals of about 20 to 40 minutes, the operation being carried on approximately three-quarters of the time at the higher range of voltages, i. e. voltages in excess of 12.5 volts.

In coatings which are formed on the aluminum or aluminum alloy, or the articles formed therefrom, I have found that there is relatively no precipitation of the metal into the electrolytic bath such as occurs in forming coatings by means of conventional processes utilizing direct current electricity. This feature of the present process permits the use of the electrolytic bath for a very much longer period of time, for once the acid concentration of the bath has been normalized it appears to continue at the normalized acid concentration during the entire operation for a considerable period of time.

Utilizing direct current, the metal decomposes and reacts with the bath to form sulphates. When the bath contains 20 grams per litre, the bath must be completely changed because of the resultant decrease in electrical conductivity of the bath. The present process is characterized by the fact that little or none of the metal is decomposed by the electrolyte and put into the bath in the form of a sulphate. This is due to the use of the relatively dilute bath which is possible by the use of the alternating current electrical energy in the process. This particular feature is one of the outstanding defects of the direct current method now being used, as this sulphate is insoluble in the bath and readily affects the conductivity of the bath, and when it reaches the concentration of 20 grams per litre of electrolyte, the bath must be changed. The efficiency of such processes of the art is progressively lessened by the rapidly diminishing conductivity value in this bath up to the ultimate point of 20 grams per litre.

The coatings formed by the process of the present invention as above described, will be found to have a substantially increased uniformity of hardness throughout the successive layers, which, when investigated by means of photomicrographs, will be shown to possess a very fine grained crystalline structure and very small and uniformly distributed pores extending therethrough. In an average case, the variation between the softest layer and the hardest layer is in the neighborhood of approximately 20%, whereas in a characteristic coating formed by the processes of the prior art, utilizing direct current electrical energy and baths of the specified concentrations of acid, there is a variation of from 140 microcharacter to approximately 5,000 microcharacter between the hardest layer and the softest layer formed.

Also, there is a considerably thicker coating

formed by means of the process herein disclosed than that of processes utilizing a flow of direct current electrical energy. In a typical example, the coating formed by the process herein described is approximately twice as thick as the coating formed by the conventional direct current processes treated for like periods of time. I believe this is due to the fact that the metal is not decomposed and changed to the sulphate as is the case in all prior operations.

A particular field in which the present invention has great utility is in the field of formed protective and oil bearing coatings on aluminum or aluminum alloy pistons for use in internal combustion engines. In this field the coatings of the present invention are superior to coatings formed by prior methods in that the coating is very much more closely knit, being formed of very much smaller particles than the coatings resulting from the direct current process. The result is that the pores of the coating are very much smaller and much more uniformly distributed than in the prior processes. This, in turn, increases the capillary value of the coating so as to give a better oil absorption of the coating than when the coating is formed by the prior processes. It is a known phenomenon that capillary elevations and depressions, other circumstances being equal, are inversely proportional to the diameters of the capillary tubes so that, considering the pores of the coating as capillary tubes having an affinity for the oil or other fluid medium, it will be seen that the smaller size of the pores and the greater uniformity of placement of the pores in the coating resulting from the present invention, will account for the greatly increased capillary values of such coating.

Excellent oxide coatings are produced under the following conditions on pistons produced from a low-aluminum high-silicon alloy which contains approximately 12% of silicon. An equal number of pistons are placed in the electrolyte and act as the electrodes. The electrolyte is composed of approximately 13% by weight of commercial sulphuric acid in aqueous solution. A 12 volt alternating current is used, one side of the line being connected to each electrode, and the 12 volt alternating current is impressed on the cell for a period of 3 minutes. The voltage is then increased to 24 volts and the treatment is continued for an additional 20 minutes, while maintaining the bath temperature at between approximately 70° to 74° F.

Using this particular alloy, the thickness of the coating will be not less than .0004 inch in thickness and the abrasimeter values will read 30 or more.

For purposes of comparison, it is interesting to note that similar coatings formed by conventional methods utilizing direct current and a stronger electrolyte, where the article is treated for the same length of time, produces coatings having an average thickness of .000327 inch as against the average thickness of the coatings produced by the use of the alternating current of .000746 inch; and the abrasimeter values will be less than 30.

In treating the aluminum or aluminum alloy articles by the present process, I find that it is possible to dispense with the preliminary cleaning and washing processes which are common to the prior art, it being sufficient with the improved process of the present invention to merely dip the aluminum or aluminum alloy article in a hot water bath. This is possible, in my opinion,

because of the use of the alternating current in the present process which, in conjunction with the electrolyte, reacts in such a way as to in effect clean the articles more completely and thoroughly than it would be possible to do by previously suggested methods. This, I believe, is due to some extent at least to the action of the alternating current in expelling the adhered surface oxygen.

10. A characteristic of the coating produced is that it is very smooth on the exterior surface so as to make possible the use of the article without using a buffering machine for the purpose of removing the chalk-like soft coating which is formed

15 by the treatment of aluminum or its alloys by conventional processes. The soft outer coating formed by conventional processes is a coating which consists, to a large extent, of the material which is precipitated into the bath as the

20 sulphate which has heretofore been described. The coating formed by the present process has no such soft outer coating and tests to date indicate that there is not more than approximately 20% variation in the microcharacter values from the outside skin of the coating to its base where it forms on the aluminum or the aluminum alloy.

Due to the action of the alternating current, less metal is taken away from the material undergoing treatment and thus the coating is of greater strength than coatings produced by prior methods wherein more of the metal is taken away during the processing operation.

While particular uses have been mentioned in the foregoing discussion of the apparatus and process of the present invention, it is to be understood that both the apparatus and the process are adapted to other uses than those herein particularly mentioned and may be used successfully to form protective coatings on articles which may be formed of some material other than aluminum or aluminum alloy but which may be coated with aluminum or aluminum alloy by such processes as calorizing, metal spraying, etc.

45. I claim:

1. A process of producing a protective coating having a thickness in excess of approximately .0004 inch and a hardness in excess of approximately 30 grams abrasimeter value, on an aluminum-silicon alloy which contains approximately 12% of silicon having substantially increased uniformity of hardness throughout the successive layers, which comprises immersing the articles formed of said alloy in an electrolytic bath containing 13% by weight of sulphuric acid in aqueous solution, electrically connecting

the immersed articles in parallel with a source of alternating current electrical energy and utilizing the immersed articles as both the anode and cathode of the circuit, and subjecting said articles to a flow of alternating current electrical energy in successive stages beginning at approximately 9 to 12.5 volts intensity for a period of approximately 3 minutes duration and increasing through successive stages to approximately 24 volts for a period of approximately 20 minutes duration at the conclusion of the process.

2. A process of producing a protective coating on an aluminum-silicon alloy containing approximately 12% silicon having substantially increased uniformity of hardness throughout the successive layers, which comprises immersing the aluminum alloy in an electrolytic bath containing 13% by weight of sulphuric acid in aqueous solution, electrically connecting the immersed alloy in parallel with a source of alternating current electrical energy and utilizing the immersed alloy as both the anode and cathode of the circuit through the bath, and subjecting the said alloy to a flow of alternating current electrical energy in successive stages beginning at approximately 9 to 12.5 volts for a period of approximately 3 minutes and thereafter increasing to approximately 20 to 24 volts for a period of approximately 20 minutes while agitating the bath to maintain a substantially constant circulation thereof and maintaining a substantially constant temperature of the bath between approximately 70° and 74° Fahrenheit.

3. A process for forming a finished and smooth unbuffed protective coating having a thickness in excess of .0004 inch and a hardness in excess of approximately 30 grams abrasimeter value on an aluminum-silicon alloy containing approximately 12% silicon having substantially increased uniformity of hardness throughout the successive layers, which comprises immersing said alloy in an oxidizing bath containing 13% by weight of sulphuric acid in an aqueous solution and passing an electrical current therethrough for a period of approximately 3 minutes duration at a potential of approximately 9 to 12.5 volts and thereafter for a period of approximately 20 minutes duration at a potential of approximately 24 volts, utilizing the said alloy in the bath as both the anode and cathode of the circuit through the bath, while agitating the bath and maintaining therein a substantially constant temperature of between approximately 70° and 74° Fahrenheit.

FRED A. WALES. 55